

Oct. 16, 1928.

1,687,486

P. A. E. ARMSTRONG

FERROUS ALLOY

Filed Aug. 14, 1925



% of Cr + appreciable quantity  
of Tantalum and with 1% - 4.5% of Silicon

INVENTOR  
P.A.E. Armstrong  
BY J. H. Dyke

ATTORNEY

## UNITED STATES PATENT OFFICE.

PERCY A. E. ARMSTRONG, OF NEW YORK, N. Y.

## FERROUS ALLOY.

Application filed August 14, 1925. Serial No. 50,255.

My invention relates to ferrous alloys that have their principal use as heat resisting parts which are required to resist progressive scaling at high temperatures, coupled with great strength at high temperatures, yet can be readily worked, machined and forged or cast into convenient shapes. Their principal applications are for valves and valve parts for internal combustion engines and for superheated steam, cast parts for annealing boxes, carburizing containers, mixing paddles, either forged or cast, for the alkali industry, and blades and rotors for gas turbines and boosters.

15 My alloy contains essentially iron, chromium, tantalum, and silicon.

My chromium range is from 1% to 20%, tantalum from an appreciable quantity to about 10%, and silicon up to about 4.5%, 20 carbon under 1.25%.

The figure of the accompanying drawing shows the approximate limits of carbon which can be used with a corresponding percentage of chromium together with tantalum 25 and silicon. Compositions having such elements within the carbon and chromium area A on said drawing are embraced within the present invention.

The higher the content of the alloying materials—except carbon—with the iron, the greater is the resistance to rust formation or surface discoloration. These properties, however, are not of major importance as respects my present invention, which is primarily intended for those applications where heat is encountered sufficient to discolor the effective working part of the surface.

For automobile engine valves I prefer the carbon about .20% to .60%; for containers, 30 low carbon under .20%; for those purposes where hardness arising from high carbon is essential, carbon about 1% to 1.10%. Steam valves subjected to high pressure and high temperature are preferably made with high 35 carbon, such as given above for valves for internal combustion engines. Such high carbon can be used to particularly good advantage when the chromium is carried to the high side of my limit.

40 The silicon content adds materially to the scale resisting property of the alloy, as for example, the temperature at which an alloy steel containing carbon .25%, chromium 1.5%, silicon .25%, materially scales is about 45 1300 degrees F. If 4% silicon is added the

scaling point temperature is about 1700 degrees F.

Chromium also raises the scale resisting temperature point. For instance, a steel containing carbon .45%, chromium 17%, silicon .25% will scale materially at about 1600 degrees F. if 2% of silicon is added the temperature at which material scaling is encountered is about 1750 degrees F.

Tantalum raises the scale resisting point. 65 For example, 2% of tantalum will raise the temperature for material scaling by about 50 to 100 degrees F.

Tantalum has an important property, which is lacking in additions of either chromium or silicon, or both, namely, tantalum increases the strength of the alloy when heated to high temperatures.

70 For example, the following table gives the approximate loads per square inch and temperatures at which test specimens of various compositions will break on a tensile testing machine.

Alloy A: C .50%, Cr 9%, Si 3.50%.

Alloy A': Alloy A with also 3% of tantalum.

Alloy B: C .35%, Cr 12%, Si .3%.

Alloy B': C .35%, Cr 12%, Si .35%, Ta 2%.

Alloy C: C .40%, Cr 3.25%, Si 3.60%.

Alloy C': C .42%, Cr 3.40%, Si 3.50%, Ta 3%.

Alloy D: C 1%, Cr 18%, Si .50%, Ta 2%.

Alloy E: C 1.07%, Cr 17.50%, Si .45%.

Alloy E': Alloy E with 8% of Ta.

| Alloy | 1200° F.          | 1400° F.         | 1550° F.         | 1650° F.        |
|-------|-------------------|------------------|------------------|-----------------|
| A     | Pounds<br>150,000 | Pounds<br>44,000 | Pounds<br>12,000 | Pounds<br>3,500 |
| A'    | 200,000           | 78,000           | 22,000           | 14,000          |
| B     | 140,000           | 52,000           | 23,000           | 20,000          |
| B'    | 240,000           | 84,000           | 40,000           | 29,000          |
| C     | 90,000            | 37,000           | 11,000           | 9,000           |
| C'    | 130,000           | 50,000           | 17,000           | 12,000          |
| D     | 230,000           | 90,000           | 50,000           | 32,000          |
| D'    | 190,000           | 65,000           | 29,000           | 24,000          |
| E     | 240,000           | 160,000          | 70,000           | 40,000          |
| E'    |                   |                  |                  |                 |

100

The temperatures given above are approximate, and as each comparison was pulled under similar conditions, the above figures can be taken as a rough guide as to the added strength imparted by the addition of tantalum. Tantalum is preferably from .25% to 3%, and more preferably from 1% to 3%.

105 The full range of chromium can be employed. I prefer to have the chromium content above 3%, and it should be above 7% if 110

it is to be subjected to severe heat conditions. For general valve purposes 8% to 9% of chromium is usually sufficient. If rust resisting conditions are encountered, the chromium content should preferably be above 7%, and may advantageously be between 12% and 17%.

The silicon content is important to the alloy when subjected to heat, and I prefer to 10 use 4% of silicon with low chromium, and about 1% of silicon with high chromium.

Valves for internal combustion engines give good results made from the following compositions:

- 15 C .45%, Cr 8.50%, Ta 3%, Si 3.25%.
- C 1%, Cr 12.50%, Ta 6%, Si 2.5%.
- C .40%, Cr 4%, Ta 2%, Si 3.5%.

Internal combustion engine valves made of ferrous alloys substantially as described do 20 not scale at high temperatures, run well and smoothly in the guides and may be hardened to resist wear on their tappet ends, making the alloy well suited for the production of integral or one-piece valves.

25 High melting point elements can be used, such as tungsten, molybdenum, columbium, vanadium, zirconium, titanium, cobalt, nickel. Nickel generally adds to the strength of the material at 1400 degrees F. and upwards, 30 but makes the material hot short at around 2200 degrees F. It also does not add to the strength of the alloy at atmospheric temperatures. Nickel is preferred low.

The high melting point metals are desired 35 under 5%. They can, however, be used in part for the tantalum, particularly tungsten, molybdenum and columbium.

40 My alloy is, of course, resistant to salt water and hot water atmospheres, to nitric acid, and dilute acids, such as citric, acetic, malic, particularly when the chromium content is increased and the carbon is decreased.

45 My alloy can be readily hardened if the carbon content is raised toward the upper limit, the higher the chromium, the more the carbon required to impart hardness by heat treatment. About 1900 degrees F. will generally be sufficient temperature, coupled with

quenching, to produce hardness. Annealing is advantageously done at about 1500 to 1750 50 degrees F.

55 My alloy generally contains manganese, preferably below 1.5%, and generally under .60%; phosphorus and sulfur should be kept low.

I claim:

1. Ferrous alloy resistant to fluids at elevated temperatures containing approximately chromium 9%, carbon .50%, silicon 3.5%, tantalum 3%, and the principal part of the 60 remainder iron.

2. Valves for internal combustion engines made from a ferrous alloy containing approximately carbon .45%, chromium 8.5%, tantalum 3%, silicon 3.25%, and the principal 65 part of the remainder iron.

3. Ferrous alloy resistant to rust, heat and acid, containing chromium 3%-18%, carbon .35%-1.1%, silicon 4%-1%, tantalum 2%-8%, and the principal part of the 70 remainder iron.

4. Valve for internal combustion engines made from ferrous alloy containing carbon .4%-1%, chromium .4%-12.5%, silicon 4%-2%, tantalum 2%-6%, and the principal 75 part of the remainder iron.

5. Ferrous alloy of high strength and resistance to scaling at high temperatures containing chromium about 1%-20%, silicon about 4%-1%, carbon from enough to produce material hardening up to about 1.25%, tantalum about .25%-3%, and the principal 80 part of the remainder iron.

6. Valves for internal combustion engines of alloy according to claim 5. 85

7. Ferrous alloy of high strength and resistance to scaling at high temperatures containing chromium about 3%-10%, silicon about 4%-1%, carbon about .30%-1%, tantalum about 1%-3%, and the principal part 90 of the remainder iron.

8. One-piece valves for internal combustion engines of alloy according to claim 7.

In testimony whereof, I have signed my name hereto.

PERCY A. E. ARMSTRONG.